

## UNITED STATES PATENT OFFICE

2,448,093

## PENETRATING OIL COMPOSITIONS

Lewis D. Gittings, Anniston, Ala., assignor to  
 Monsanto Chemical Company, St. Louis, Mo.,  
 a corporation of Delaware

No Drawing. Application October 24, 1945,  
 Serial No. 624,316

6 Claims. (Cl. 252—59)

1

This invention relates to oily compositions having outstanding penetrating and creeping properties and to a process of producing same.

An object of the invention is to provide a combined penetrating and lubricating oil characterized by having a high degree of capillarity which

2

with dicyclohexyl, and it is prepared by simply mixing these ingredients together since they are freely soluble in each other.

Reference is made to the following table which illustrates a number of typical compositions prepared in accordance with the present invention.

## Penetrating oil compositions

| Com. No. | Dicyclohexyl,<br>Per Cent By<br>Vol. | Kerosene<br>Per Cent By<br>Vol. | SAE 10 Oil,<br>Per Cent By<br>Vol. (A) | Spindle Oil A<br>Per Cent By<br>Vol. (B) | Viscosity at<br>100° F. Say-<br>bolt Universal<br>Seconds | Specific<br>Gravity<br>at 25° C. | Flash<br>Point<br>° F. |
|----------|--------------------------------------|---------------------------------|----------------------------------------|------------------------------------------|-----------------------------------------------------------|----------------------------------|------------------------|
| 1        | 50                                   |                                 | 50                                     |                                          |                                                           |                                  |                        |
| 2        | 60                                   |                                 | 40                                     |                                          |                                                           |                                  |                        |
| 3        | 25                                   | 25                              | 50                                     |                                          |                                                           |                                  |                        |
| 4        | 60                                   | 35                              | 5                                      |                                          |                                                           |                                  |                        |
| 5        | 5                                    | 20                              |                                        | 75                                       | 34.8                                                      | 0.852                            | 170.6                  |
| 6        | 10                                   | 15                              |                                        | 75                                       | 56.2                                                      |                                  | 220                    |
| 7        | 15                                   | 15                              |                                        | 70                                       | 56.2                                                      |                                  | 235                    |
|          |                                      |                                 |                                        |                                          | 53.2                                                      |                                  | 215                    |

causes it to quickly penetrate and lubricate coherent or coalesced surfaces.

Another object of the invention is to provide a penetrating oil which is highly effective for loosening badly rusted nuts, bolts, studs, and similar so called "frozen connections."

An additional object is to provide a penetrating oil characterized by its ability to loosen or dissolve rust or corrosion which prevents relative movement between metal surfaces.

A further object is to provide a novel composition which, by virtue of its pronounced penetrating powers, is adapted for use in the removal of carbon from internal combustion engines.

Other objects will be apparent to those skilled in the art as the description proceeds.

A penetrating oil to be of commercial value must have a high degree of capillarity so that it will quickly work its way into minute spaces between corroded, rusted or "frozen" surfaces. It must also have a low viscosity and a high preferential wetting power for the surface to be lubricated as it is essential that the oil penetrate the rust and adhere to the underlying surface. Moreover, where the penetrating oil is to be used as a lubricant it must have a vapor pressure such that after reaching its point of use, it will not completely evaporate and it must also have sufficient body to lubricate the metal surfaces when relative motion occurs.

I have developed a composition fully satisfying the above requirements which is characterized by outstanding penetrating and creeping properties. This composition comprises a light hydrocarbon oil or a mixture of a light hydrocarbon oil and a lubricating oil in combination

## (A) Properties of SAE-10 oil:

|    |                                |         |
|----|--------------------------------|---------|
| 20 | A. P. I. gravity @ 60° F. min. | 30.5    |
|    | Color, Robinson                | 8-9     |
|    | Open flash °F. ASTM min.       | 410     |
|    | Pour test °F. max.             | —20     |
| 25 | Viscosity @ 100° F. Say        | 185/195 |
|    | Per cent Conradson carbon max. | 0.12    |
|    | V. I. min.                     | 105     |

## (B) Properties of spindle oil A:

|    |                              |    |
|----|------------------------------|----|
| 30 | Viscosity at 100° F. seconds | 72 |
|----|------------------------------|----|

30 The above compositions are highly efficient penetrating oils and may be used for loosening rusted nuts, bolts, studs, laboratory ring stands and other so called "frozen connections." Of the above compositions, Example 4 is preferred since it possesses exceptional penetrating properties and has been found superior to any of the commercial penetrating oils now on the market.

35 Compositions 3, 5, 6 and 7 are efficient lubricants and in addition have excellent penetrating powers, but in the latter respect they are not quite as effective as composition 4.

40 All of the foregoing compositions, and particularly composition 4, are adapted for use in the removal of carbon from internal combustion engines. When employed for this purpose, the compositions are introduced into the engine through the carburetor air-intake while the engine is in operation. The amount added varies with the composition selected and with the condition and size of the engine, but in general substantially complete removal of carbon can be obtained by means of about one pint of penetrating oil. As an alternative to the above procedure, the penetrating oil may be added directly to the

55 motor fuel.

In place of kerosene, other materials such as light hydrocarbons (28.0° A. P. I. gravity or higher), "Varnolene," furnace oil, gasoline, light gas oil, one of the pressure naphthas (in the refined or crude state) or mixtures of two or more of these may be employed.

Moreover, other lubricants may be substituted for those specifically mentioned in the above table, such as:

1. Spindle oil having a Saybolt viscosity of from about 70 to 350 seconds and preferably from 90 to 130 seconds at 100° F.

2. Lubricating oils having a specific gravity of about 0.89 to 0.91.

3. Lubricating oil of a paraffinic or an asphaltic base with a viscosity of about 100° Saybolt at 100° F.

4. Light lubricating oils of 20° A. P. I. gravity or lighter.

The proportions of the various ingredients may fluctuate over wide limits without departing from the spirit of the present invention, it being understood that this factor will vary depending upon the viscosity of the light hydrocarbon oil and/or the lubricating oil and the work to be done.

For example, the amount of dicyclohexyl may vary from 5% to 60% by volume, and even higher percentages are within the scope of the invention but for a penetrating oil of general utility I prefer to employ about 60% by volume of this compound.

The content of light hydrocarbon oil and lubricating oil is preferably maintained within the ranges of from 5% to 35% and 15% to 75% by volume respectively, but higher or lower proportions of these materials are also within the scope of the invention. In general, where the composition is employed as a combined penetrating and lubricating oil, it is desirable to use a relatively high proportion of lubricating oil in relation to the light hydrocarbon oil. On the other hand if a penetrating oil of pronounced creeping properties is desired, the proportion of light hydrocarbon oil should be increased and the content of lubricating oil should be correspondingly decreased.

The foregoing description has been restricted to combinations of dicyclohexyl with light hydro-

carbon oils and/or lubricating oils, but it should be clearly understood that the invention is not limited thereto as dicyclohexyl increases the effectiveness of penetrating oils generally. Thus, in its broadest aspect, the present invention contemplates the addition of dicyclohexyl to all known penetrating oils to increase their efficiency either by replacing or supplementing the active constituent thereof.

While I have described my invention in detail, it should be understood that many changes may be made therein without departing from the spirit of same.

What I claim is:

1. A penetrating oil comprising in combination a hydrocarbon oil and from 5% to about 60% by volume of dicyclohexyl.
2. A penetrating oil comprising in combination a low boiling petroleum oil, a lubricating oil and from 5% to 60% by volume of dicyclohexyl.
3. A penetrating oil comprising in combination kerosene, a low viscosity lubricating oil and from 5% to 60% by volume of dicyclohexyl.
4. A penetrating oil comprising in combination 35% by volume of kerosene, 5% by volume of a low viscosity lubricating oil and 60% by volume of dicyclohexyl.
5. A combined penetrating and lubricating oil comprising in combination 20% by volume of kerosene, 75% by volume of a low viscosity lubricating oil and 5% by volume of dicyclohexyl.
6. A combined penetrating and lubricating oil comprising in combination 25% by volume of kerosene, 50% by volume of a low viscosity lubricating oil and 25% by volume of dicyclohexyl.

LEWIS D. GITTINGS.

#### REFERENCES CITED

The following references are of record in the file of this patent:

#### UNITED STATES PATENTS

| Number    | Name      | Date           |
|-----------|-----------|----------------|
| 1,333,363 | Abbott    | Mar. 9, 1920   |
| 1,580,233 | Copthorne | Apr. 13, 1926  |
| 1,822,886 | Elderkin  | Sept. 15, 1931 |
| 2,389,608 | Calva     | Nov. 27, 1945  |